

## UNITED STATES PATENT OFFICE

ELMER J. WALTZ, OF RIVERSIDE, NEW JERSEY

## CHROMIUM PLATING

No Drawing.

Application filed January 21, 1929. Serial No. 334,131.

My invention relates to electrolytic deposition of chromium and more particularly to a process of electroplating with chromium and a bath or aqueous solution for use in connection therewith.

One object of my invention is to provide, in a process for producing chromium plating, a bath characterized by its improved throwing power. A further object is to produce chromium plating of bright lustre, even density and lasting quality.

I have found that a bath containing chromic acid in water solution can be made to possess improved throwing power for chromium plating when there is liberated in the bath hydrocyanic acid (HCN) or cyanide (CN) ions. I therefore add to a bath containing chromic acid ( $\text{CrO}_3$ ) in excess, an alkaline cyanide, as for example sodium cyanide ( $\text{NaCN}$ ), which reacts to liberate hydrocyanic acid (HCN), the other product of the reaction being sodium dichromate ( $\text{Na}_2\text{Cr}_2\text{O}_7$ ).

The presence of alkaline chromates or bichromates in the chromic acid solution also improves the throwing power. Chromic acid in solution is only slightly ionized whereas alkaline chromates and bichromates are strongly ionized. Accordingly the salts resulting from the reaction produce better electrical conductivity in the bath, by virtue of the larger number of dissociate ( $\text{CrO}_3$ ) ions therein, and freer deposition of chromium is permitted.

The following constitutes the proportions of chromic acid and sodium cyanide which give the most satisfactory results:

|                |                    |
|----------------|--------------------|
| Chromic acid   | 18. oz. per gallon |
| Sodium cyanide | 1½ oz. per gallon  |
| Water          | 1 gallon           |

With this electrolyte I have found that low carbon steel anodes give excellent results. I preferably utilize as anode a steel tank though I may, of course, employ separate low carbon steel anodes on either side of the cathode in which case the distance from anode to cathode should be from two to six inches.

In carrying out my novel process, the object to be plated is first highly polished and

then placed in an alkali cleaner. When cleaned the object is rinsed in cold water and scrubbed to remove the cleaner film. I then preferably subject the object to successive baths of nickel, copper and nickel, though plating may be effected directly on copper, brass, steel or nickel. It is not necessary that the work be chemically clean preparatory to plating, but it is important that it have a highly polished surface.

The bath is prepared in accordance with the above formula and maintained at a comparatively cold temperature for best results. Good plating is obtained with an electric current of from 3½ to 6 volts and a current density in the neighborhood of 60 amperes per square foot. Under the above conditions a serviceable plate with bright lustre and uniform density may be obtained in from 1½ to 2 minutes. From time to time the electrolyte may be replenished by the addition of chromic acid, care being taken to avoid excess acid as dark tones will be caused thereby. If the bath should lack throwing power, sodium cyanide should be added in small portions until the solution contains its normal proportions.

It will be readily understood that I do not limit myself to the precise details of procedure described above and that the ratio of alkaline cyanide and chromic acid per gallon of solution used in the electrolyte may be modified within reasonable limits without departing from the spirit of my invention.

Having thus described my invention, I claim:

A bath for electrodepositing chromium containing a solution of chromic acid 18 ounces per gallon and sodium cyanide 1½ ounces per gallon.

In testimony whereof, I have hereunto signed my name at Philadelphia, Pennsylvania, this 17th day of January, 1929.

ELMER J. WALTZ.

95

100